

Jan. 1, 1957

E. B. MANCKE

2,776,207

TREATMENT OF IRON ORES

Filed April 5, 1951

2 Sheets-Sheet 1

*Fig. 1.*

*Ammonium Sulfate Process.*



INVENTOR

*Edgar B. Mancke.*

BY *R. S. C. Mougherty*

ATTORNEY

Jan. 1, 1957

E. B. MANCKE

2,776,207

TREATMENT OF IRON ORES

Filed April 5, 1951

2 Sheets-Sheet 2

*Fig. 2.*

*Sulfuric Acid Process.*



INVENTOR

*Edgar B. Mancke.*

BY *R. S. C. Mougherty*

ATTORNEY

2,776,207

## TREATMENT OF IRON ORES

Edgar B. Mancke, Bethlehem, Pa., assignor to Bethlehem Steel Company, a corporation of Pennsylvania

Application April 5, 1951, Serial No. 219,363

8 Claims. (Cl. 75—115)

This invention relates to the treatment of iron ores of the Mayari, or nickeliferous lateritic, type, and more particularly to the method of removing from such ore most of the nickel, cobalt and chromium.

The principal object of this invention is to produce, from a Mayari type ore, an iron ore product low in nickel, cobalt and chromium.

Another object is to produce an iron ore product from Mayari ore by chemical treatment wherein the treating material can be largely recovered and recycled.

The nickeliferous lateritic, or Mayari, type iron ores generally contain nickel in quantities of from 0.25 to 1.50 percent and cobalt in quantities of from 0.05 to 0.30 percent, on a calcined basis. Chromium is usually present in such ores in quantities ranging from 1.50 to 2.50 percent. In refining a Mayari type of ore, removal of nickel, cobalt and chromium presents a difficult separation problem. The separation of the nickel, cobalt and chromium from the ore is a highly important consideration, for, in certain cases, in the manufacture of carbon steel, specifications call for extremely low amounts of impurities such as nickel and chromium, and to produce a steel of this type it is necessary that the ore as charged to the blast furnace must have low nickel and chromium contents.

I have found that ores of the Mayari type, when solubilized with a sulfate and the sulfate solution subsequently subjected to an autoclave treatment, can be made to yield an iron ore product quite low in nickel, cobalt and chromium. The sulfate solution may be prepared by any feasible means, for example, the ore may be roasted and then leached with sulfuric acid or leached directly with sulfuric acid. Another method of putting the bulk of the ore in solution would be to roast the ore with ammonium sulfate, followed by a water or sulfuric acid leach. In either method of solubilization, an insoluble residue composed of most of the silica and a part of the total chromium must be separated from the solution. When ore is treated by the above-mentioned solubilization methods in such manner so that at least 85 percent of the iron, nickel and cobalt dissolves, then roughly one-third, or slightly more, of the total chromium will also dissolve.

Upon autoclaving a sulfate solution containing iron, nickel, cobalt and chromium values under suitable conditions of time, temperature and pressure, an iron product of basic iron sulfate is precipitated containing less than 0.10 percent nickel or cobalt. The amount of chromium in the iron precipitate will depend on the oxidation state of the chromium at the time of autoclaving. If the chromium is in the hexavalent state, an iron precipitate can be produced which will contain about 0.15 percent chromium or less; however, if the autoclave feed solution contains chromium which is predominantly in the trivalent state, somewhat larger quantities of chromium will be precipitated along with the iron. In any case, the ratio of iron to chromium in the precipitate will be higher than in the initial solution treated in the autoclave. Even though the solution is not oxidized, the chromium content of the product will be well under that of the ore being

treated. These larger quantities of precipitated chromium which occur with trivalent chromium may not be objectionable for some steelmaking purposes, in which case care need not be taken to oxidize prior to autoclaving. In any event, the autoclaving operation will produce an ore low in nickel. When it is desirable to produce a resultant iron ore product having chromium present in amounts less than 0.15 percent, precautions must be taken, prior to autoclaving, to secure hexavalent chromium in the feed stock. A substantial proportion of hexavalent chromium can be formed in the feed solution by roasting the ore in air prior to leaching. However, more complete oxidation can be obtained by adding an oxidizing agent such as potassium permanganate to the sulfate solution prior to autoclaving.

Roasting the ore in air is not essential with either of the above solubilizing methods. However, one advantage of roasting the ore in air is derived from the fact that improved settling and filtering properties are obtained when air roasting precedes leaching. Another advantage of air roasting the ore is that ore which has been roasted in this manner is more reactive than natural ore. For a given leaching treatment, solubilities are higher if the ore has been roasted first in the vicinity of 500° to 1200° F., 800° F. being particularly effective. These advantages are evident not only with subsequent acid leaching, but also when an air roast is followed by a solubilizing ammonium sulfate roast and a leach.

One method by which an iron ore product, low in nickel and chromium, can be obtained from a Mayari type of ore by my invention would be to give the ore an oxidizing roast at approximately 800° F. The oxidizing roast is followed by a second roast in which the pre-roasted ore is treated with ammonium sulfate at about 800° F. until iron, nickel, cobalt and combining chromium are in the form of sulfates. Ammonia gas is liberated in this second roast and collected for use in the process at a later stage, as will be explained. The sulfates of iron, nickel, cobalt and chromium, as well as some manganese and aluminum are leached with water. Alternatively, the leach may be made with an aqueous solution of sulfuric acid. After leaching, the insoluble residue is separated from the solution, as by filtration. The residue contains silica and insoluble chromium compounds. This residue may be utilized in refractories if desired. The leach solution is then autoclaved at suitable temperature and for a time sufficient to produce a precipitate of basic iron sulfate, most of the nickel, cobalt and chromium remaining in solution. After the completion of the autoclave treatment, the basic iron sulfate precipitate is separated from the remaining solution, preferably by filtration, and the precipitate leached with ammonium hydroxide. The ammonium hydroxide used at this juncture can be prepared from the ammonia gas liberated during the ammonium sulfate roasting operation. The hydroxide leach removes sulfur from the basic iron sulfate in the form of ammonium sulfate, leaving an iron product of ferric oxide low in nickel, cobalt and chromium. The basic iron sulfate normally contains approximately 18 percent sulfur, while, after leaching with ammonium hydroxide, the sulfur in the remaining iron oxide ore product will be below 2 percent. The ammonium sulfate recovered from the ammonium hydroxide leaching step can be recycled to the ammonium sulfate roasting operation.

As has been stated, the solution after the autoclaving operation contains most of the nickel, cobalt and the soluble chromium. The solution also contains manganese and aluminum sulfates and part, possibly 20 percent, of the original iron. Either all or part of this solution may be used for the recovery of the valuable metals it contains. If desired, part of the solution may be returned to the ammonium sulfate roasting operation, or to the

leaching step immediately following roasting. A further alternative lies in liberating sulfur oxide gases from the solution, and using the sulfur gases in the acid leach step, either directly as the gas, or after reforming sulfuric acid from them, if the acid leach is made part of the process.

While the method outlined above produces a satisfactory end product of iron ore low in nickel, cobalt and chromium, an optional method of performing the same may be preferred in some situations, dependent on equipment and handling factors. Instead of pre-roasting the ore to obtain hexavalent chromium in the leaching step, the sulfate leach solution is oxidized with a permanganate or other oxidizing compound prior to autoclaving. Either method of oxidizing the soluble chromium insures an iron ore end product low in chromium. Additionally, pre-roasting may be used in conjunction with further oxidation of the leach solution. It has been found that when treating ore with both an oxidizing pre-roast and a subsequent oxidizing step upon the ore in solution, more iron dissolves in the leaching step because the ore is more reactive, thus more of the iron tends to be precipitated in the autoclaving step, and less oxidizer is required for the reason that the pre-roasting step accomplishes part of the oxidation. In addition, settling and filtering properties of the precipitated iron are improved by the pre-roast.

In the accompanying flow chart, Fig. 1, there is illustrated diagrammatically the process hereinbefore described.

As one specific example wherein my invention may be performed, a Mayari type ore having the following general analysis:

|                                                | Average, percent | Range, percent |
|------------------------------------------------|------------------|----------------|
| Iron (Fe)-----                                 | 55               |                |
| Nickel (Ni)-----                               | 1.0              | 0.25 to 1.56   |
| Chromium (Cr)-----                             | 2.2              | 2.1 to 2.3     |
| Cobalt (Co)-----                               | 0.15             | 0.05 to 0.35   |
| Manganese (Mn)-----                            | 0.5              | 0.24 to 1.76   |
| Silica (SiO <sub>2</sub> )-----                | 5.0              | 1.6 to 7.0     |
| Alumina (Al <sub>2</sub> O <sub>3</sub> )----- | 10.0             | 6.0 to 14.0    |

is pre-roasted in air at 800° F. for four hours. The pre-roasted ore is then roasted with ammonium sulfate at 800° F. for four hours to solubilize iron, nickel, cobalt, part of the chromium, and manganese and aluminum. The thus roasted ore is then leached with an aqueous solution of sulfuric acid and the soluble metal values extracted. After separating the insoluble residue from the sulfate solution, the solution is subjected to an oxidizing treatment by the addition of potassium permanganate. The oxidized solution is then autoclaved for one hour at 400° F. during which about 80 percent of the iron, previously in solution will be precipitated in the form of basic iron sulfate. After separating the precipitate from the remaining autoclave solution and thoroughly washing, the precipitate is leached with ammonium hydroxide (formed from ammonia gas produced in the ammonium sulfate roasting step), and an iron oxide ore product remains which has a nickel content of less than 0.10 percent, and chromium in an amount less than 0.15 percent. A typical example of an ore product made by my method analyzed as follows:

|                                                |                          |
|------------------------------------------------|--------------------------|
| Iron (Fe)-----                                 | 68.7% (calcined basis).  |
| Nickel (Ni)-----                               | 0.03 (calcined basis).   |
| Cobalt (Co)-----                               | < 0.01                   |
| Chromium (Cr)-----                             | 0.08 (calcined basis).   |
| Manganese (Mn)-----                            | < 0.10 (calcined basis). |
| Alumina (Al <sub>2</sub> O <sub>3</sub> )----- | 0.90 (calcined basis).   |
| Silica (SiO <sub>2</sub> )-----                | < 1.00 (calcined basis). |
| Sulfur (S)-----                                | 1.40 (dry basis).        |

Another mode of performing my invention would be to give the ore an oxidizing roast and then leach the

roasted ore with strong sulfuric acid to solubilize iron, nickel, cobalt, most of the soluble chromium, and manganese and aluminum. After separating the insoluble residue from the solution formed during leaching, said solution is introduced into an autoclave, either with or without further oxidation of the solution prior to the autoclaving step. Whether or not further oxidation is required will be determined by the sufficiency of the oxidizing roast, and the amount of chromium which can be tolerated in the product. After autoclaving the solution under suitable conditions of time, temperature and pressure, the resultant slurry is withdrawn, and the precipitated basic iron sulfate is separated from the remaining solution. The solution at this point contains most of the nickel, cobalt, the leach soluble chromium, manganese and aluminum, along with about 20 percent of the soluble iron. To obtain an iron ore product comparable to that obtained when an ammonium sulfate roast is used, as described in the previous example, the basic iron sulfate may be roasted to drive off sulfur oxide gases and leave an iron oxide low in nickel, cobalt and chromium. The sulfur oxide gases (SO<sub>2</sub> and SO<sub>3</sub>) may be returned to the leaching operation.

In the accompanying flow chart, Fig. 2, there is a diagrammatic illustration of a method of performing my invention by use of a strong sulfuric acid leach, with subsequent treatment for the recovery of an iron oxide ore product by roasting.

In a specific example of performing my invention according to the process outlined in the accompanying flow chart, Fig. 2, an ore sample, having the same general analysis as that given for the sample of the previous example, is roasted in air at 800° F. and then leached with 40 percent (weight) sulfuric acid to solubilize most of the iron, nickel, cobalt, manganese, aluminum and soluble chromium. Upon the completion of the leach, the insoluble residue containing silica and part of the chromium is separated from the solution. The solution is then oxidized with potassium permanganate to insure oxidation of chromium to the hexavalent state, after which the solution is introduced into an autoclave. The autoclaving operation may be performed at a temperature of 400° F. for one hour. During autoclaving, about 80 percent of the original iron will be precipitated in the form of basic iron sulfate, the other metal values present remaining in solution except for incidental and unharful amounts which form part of the iron precipitate. After separating the precipitate from the remaining autoclave solution and thoroughly washing, the basic iron sulfate is roasted to convert it to iron oxide, the sulfur gases produced being collected, regenerated to sulfuric acid, and returned to the sulfuric acid leaching step. Regeneration of the sulfur gases to sulfuric acid before use in leaching may not be necessary in every case, for the gases may be introduced directly into the leaching solution. A typical example of an iron oxide ore product, made by the method of the foregoing, had the following analysis:

|                                                |                          |
|------------------------------------------------|--------------------------|
| Iron (Fe)-----                                 | 68.7% (calcined basis).  |
| Nickel (Ni)-----                               | 0.03% (calcined basis).  |
| Cobalt (Co)-----                               | <0.01% (calcined basis). |
| Chromium (Cr)-----                             | 0.11% (calcined basis).  |
| Manganese (Mn)-----                            | <0.10% (calcined basis). |
| Alumina (Al <sub>2</sub> O <sub>3</sub> )----- | 0.82% (calcined basis).  |
| Silica (SiO <sub>2</sub> )-----                | <1.00% (calcined basis). |

In the example just given, the air roast at 800° F., prior to acid leaching, so conditions the ore that a considerable quantity of the dissolved chromium will be in the hexavalent state after leaching. Depending on the ultimate use of the resultant ore product, further oxidation of the chromium may be unnecessary. However, when an ore product is desired having the lowest possible amount of chromium, it is necessary to oxidize the solution containing the metal values prior to autoclaving.

In performing my invention, the method to be used

to solubilize the metal values and to remove sulfate radicle from the basic iron sulfate will depend primarily on operating considerations and on the type of solubilizing medium preferred in any individual case. The resultant iron ore product will be of the same general character and quantity in either of the proposed methods shown in the flow charts. It is desirable, however, in order to fully realize on the economic possibilities of the invention, that, whichever method of sulfation is used, the sulfating material be recovered. As has been shown in the example in which an ammonium sulfate roast is used, ammonia gas recovered from the roasting operation is used to form ammonium hydroxide for leaching the precipitated basic iron sulfate. The ammonium sulfate formed in the reaction which accompanies leaching of the basic iron sulfate is returned to the ammonium sulfate roasting step. In this manner a closed circuit is maintained in respect to both the ammonia ( $\text{NH}_4$ ) and the sulfate ( $\text{SO}_4$ ) radicle, and by recycling the reformed ammonium sulfate to the ammonium sulfate roasting step most of the sulfating material recovered, the original charge of ammonium sulfate being constantly available for re-use in the treatment of fresh ore.

Likewise, when the means of sulfation is that of an air roast accompanied by a sulfuric acid leach, roasting of the precipitated basic iron sulfate to recover sulfur oxide gases, and eventually recycling the gases in the form of sulfuric acid to the leach, provides a means of recovery of sulfating material whereby only water and make-up reagent need be added to maintain the proper leaching conditions during subsequent treatment of fresh batches of ore. Here, again, it should be noted that regeneration of the sulfur gases to sulfuric acid before use in leaching may not be necessary in every case; the gases may be introduced directly into the leach solution, if desired.

I have found that while the autoclaving conditions given in each of the above examples give excellent separation of the iron from the non-ferrous metal values, the conditions are meant as examples only, for the temperature during autoclaving may be varied through quite a broad range, the practical temperature being in the vicinity of 390° to 420° F. At lower temperatures, e. g., 350° F., only a small part of the iron will precipitate, making the process impractical. Temperatures higher than 400° F. are effective but temperatures very much higher than 400° F., while effective to precipitate iron from solution offer some practical difficulties because of the very high pressures which are then needed.

It should be pointed out that good nickel separations and quite good chromium separations can be made by the proposed methods even though care is not taken to assure the oxidation of the sulfate solution prior to autoclaving; however if an iron ore product very low in both nickel and chromium is desired, most of the chromium in the sulfate solution prior to autoclaving must be oxidized to the hexavalent state.

In the autoclave reaction, and in those which follow the autoclaving step, cobalt has been found to respond in a manner similar to that of nickel, therefore any remarks as to the action of nickel made herein will apply equally as well to cobalt.

I claim:

1. A method of treating nickeliferous, lateritic iron ore containing chromium to obtain an iron ore product low in nickel, cobalt and chromium which comprises roasting the ore under oxidizing conditions at from between 500° to 1100° F., dissolving metal values of the ore by leaching the roasted ore with an aqueous liquid which contains a sulfur compound of the group consisting of sulfuric acid, sulfur trioxide, sulfur dioxide and mixtures thereof, separating the solution formed during the leaching operation from the residue, oxidizing said separated solution to convert a substantial portion of the chromium to the hexavalent state, autoclaving said separated solution at a temperature of not less than about 390°

10  
15

6. to precipitate basic iron sulfate thus producing a slurry, separating the slurry liquid from the precipitated basic iron sulfate.

2. A method of treating a nickeliferous, lateritic iron ore containing chromium to obtain an iron ore product low in nickel, cobalt and chromium which comprises roasting the ore with ammonium sulfate, dissolving metal values of the ore by leaching the roasted ore with water, separating the solution formed during the leaching operation from the residue, oxidizing said separated solution to convert a substantial portion of the soluble chromium to the hexavalent state, autoclaving the oxidized solution at a temperature of not less than about 390° F. to precipitate basic iron sulfate thus producing a slurry, separating the slurry liquid from the precipitated basic iron sulfate.

3. A method of treating a nickeliferous, lateritic iron ore containing chromium to obtain an iron ore product low in nickel, cobalt and chromium which comprises roasting the ore with ammonium sulfate, dissolving metal values of the ore by leaching the roasted ore with an aqueous solution containing sulfuric acid, separating the solution formed during the leaching operation from the residue, oxidizing said separated solution to convert a substantial portion of the soluble chromium to the hexavalent state, autoclaving the oxidized solution at a temperature of not less than about 390° F. to precipitate basic iron sulfate thus producing a slurry, separating the slurry liquid from the precipitated basic iron sulfate.

4. A method of treating a nickeliferous, lateritic iron ore containing chromium to obtain an iron ore product low in nickel, cobalt and chromium which comprises pre-roasting the ore under oxidizing conditions at from between 500° to 1100° F., roasting the pre-roasted ore with ammonium sulfate, leaching the roasted ore with water, separating the solution formed during the leaching operation from the residue, oxidizing said separated solution to convert a substantial portion of the soluble chromium to the hexavalent state, autoclaving said separated solution at a temperature of not less than about 390° F. to precipitate basic iron sulfate thus producing a slurry, separating the slurry liquid from the precipitated basic iron sulfate.

5. A method of treating a solution containing iron and chromium sulfates which comprises oxidizing the solution to convert a substantial part of the chromium to the hexavalent state, autoclaving the oxidized solution at a temperature of not less than about 390° F. to precipitate an iron compound having an iron to chromium ratio considerably higher than the iron to chromium ratio of said solution.

6. A method of treating a nickeliferous lateritic iron ore containing chromium to obtain an iron ore product low in nickel and chromium, which comprises sulfating the chromium, nickel and iron and dissolving the sulfates to form an aqueous solution of such values, separating the solution from the residue, oxidizing said separated solution to convert a substantial portion of the chromium to the hexavalent state, autoclaving the solution at a temperature of not less than 390° F. to precipitate an iron compound, and separating the solution containing nickel and chromium from the precipitated iron compound.

7. A method of treating a nickeliferous lateritic iron ore containing chromium to obtain an iron ore product low in nickel and chromium, which comprises subjecting the ore to an oxidizing roast, sulfating the chromium, nickel and iron and dissolving the sulfates to form an aqueous solution of such values, separating the solution from the residue, oxidizing said separated solution to convert a substantial portion of the chromium to the hexavalent state, autoclaving the solution at a temperature of not less than 390° F. to precipitate an iron compound and separating the solution containing nickel and chromium from the precipitated iron compound.

75

8. A method of treating nickeliferous, lateritic iron ore containing chromium to obtain an iron ore product low in nickel, cobalt and chromium which comprises dissolving metal values of the ore by leaching with an aqueous liquid which contains a sulfur compound of the group consisting of sulfuric acid, sulfur trioxide, sulfur dioxide and mixtures thereof, separating the solution formed during the leaching operation from the residue, oxidizing said separated solution to convert a substantial portion of the soluble chromium to the hexavalent state, autoclaving said oxidized solution at a temperature of not less than about 390° F. to precipitate basic iron sulfate thus producing a slurry, and separating the slurry liquid from the precipitated basic iron sulfate.

15

|              |                 |                |
|--------------|-----------------|----------------|
| 1,403,237    | Eustis          | Jan. 10, 1922  |
| 1,487,145    | Caron           | Mar. 18, 1924  |
| 1,489,347    | Davison         | Apr. 8, 1924   |
| 1,582,347    | Read            | Apr. 27, 1926  |
| 5 2,005,120  | Whetzel         | June 18, 1935  |
| 2,098,056    | McBerty         | Nov. 2, 1937   |
| 2,296,423    | Clark           | Sept. 22, 1942 |
| 2,357,715    | Westby          | Sept. 5, 1944  |
| 10 2,402,103 | Udy             | June 11, 1946  |
| 2,430,261    | Udy             | Nov. 4, 1947   |
| 2,435,304    | Foerster et al. | Feb. 3, 1948   |
| 2,520,958    | Poole et al.    | Sept. 5, 1950  |
| 2,584,700    | Hayward         | Feb. 5, 1952   |
| 2,670,271    | Thomsen         | Feb. 23, 1954  |

## References Cited in the file of this patent

## UNITED STATES PATENTS

|           |                  |               |
|-----------|------------------|---------------|
| 981,451   | McKechnie et al. | Jan. 10, 1911 |
| 1,237,765 | Eustis           | Aug. 21, 1917 |
| 1,258,934 | Nitchie          | Mar. 12, 1918 |
| 1,364,573 | Moore            | Jan. 4, 1921  |

20

Standard Methods of Chemical Analysis, by Scott, 4th edition, vol. 1, pp. 249, 250. Pub. by D. Van Nostrand Co., Inc., New York, 1925.

"A Comprehensive Treatise on Inorganic and Theoretical Chemistry," by Mellor, vol. 14, pub. by Longmans, Green and Co., 1935, page 323.

## OTHER REFERENCES